# EUROPEAN PATENT SPECIFICATION

(11) **EP 1 360 401 B1**
(45) Date of publication and mention of the grant of the patent: **03.05.2006**
(21) Application number: 02703840.5
(22) Date of filing: 07.02.2002
(51) Int. Cl.: F01N 1/24

(54) **SOUNDPROOFING MATERIAL FOR EXHAUST SILENCERS THAT EXPANDS AT A CERTAIN TEMPERATURE**
SCHALLDÄMPFENDES MATERIAL FÜR ABGASSCHALLDÄMPFER, DAS BEI EINER BESTIMMTEN TEMPERATUR EXPANDIERT
MATERIAU D'INSONORISATION POUR SILENCIEUX DE REFOULEMENT SE DILATANT A UNE CERTAINE TEMPERATURE

(30) Priority: 13.02.2001 IT NA20010011
(43) Date of publication of application: 12.11.2003
(73) Proprietor: Klevers Italiana S.R.L., 80022 Arzano (IT)
(72) Inventor: ESPOSITO, Gerardo, Ciro, I-80079 Procida (IT)
(74) Representative: TBK-Patent
(86) International application number: PCT/IT2002/000077
(87) International publication number: WO 2002/066800

(56) References cited:
- WO-A-99/23367
- US-A- 4 077 491
- US-A- 6 155 379

## Description

The present state of art for internal combustion engines' silencer construction in the automotive and motorcycling field, makes a large use of fiber glass because of its excellent soundproofing property.

The fiber glass is inserted, during the silencer's working process, in the interspace between the exhaust pipe and the external covering (aluminium, carbon, titanium, steel and similar) simply pressing inside the interspace a predetermined weight of fiber glass or needled mat.

This working process doesn't allow an homogeneous and even distribution of the fiber; in other words we may have somewhere an absence of material that could cause an heat escape damaging the silencer's external covering with the consequent reduction of acoustic efficiency. Is known the document WO9923367A which discloses a soundproofing and lagging material in which the yarns are sewed with synthetic yarns. When the synthetic yarns burn the fiber glasses, arranged parallel one another, are released and are free to move conditioned only by the pressure and/or by gravity; so they may cause somewhere an absence of material.

Is well-know, also the document US6/55379A, which discloses a multidirectional yarns overlopping; the layers are hold together by resins and not by yarns.

When the resins dissolve themselves the layers don't increase their volume; the weight necessary in order to filling the whole available cavity is excessive; moreover the yarns, with the vibration, tend to extend themselves.

The present industrial invention purpose is to propose a material that allows a correct disposition and an homogeneous insulation inside the silencer.

The right material for this application has been obtained by the solution idea that is object of the present industrial invention, which consists of a particular weaving process of : fiber glass yarn, treated for high temperature, aramid fiber, synthetic, steel and inconel.

This kind of weaving consists of the disposition of this fiber at 90°, at +45° and at -45°, so that we can obtain a traction and disposition homogeneity and also an even insulation.

The yarns, arranged in this way, are compacted and hold together by synthetic or natural fiber, arranged at variable distance.

The particular yarns and stitching disposition is shown on the enclosed plate.

With reference to it, the fiber glass yarns, arranged horizontally, are indicated with (1); on them are overlapped the yarns (2), made of fiber glass and arranged orthogonally to the precedent yarns.

Then, the yarns (3) and (4) are overlapped on the two wefts forming an angle of about +45° and -45° with the horizontal yarn.

The yarns so overlapped and compacted are sewed with synthetic or cotton yarns (5), preferably arranged parallel to (1).

The sewing yarn isn't heat - resistant, so, when it is struck by the heat flow, it's burned in a few time, releasing the compacted yarns which increase their volume.

These yarns, even if they have increased their volume, will maintain a controlled and homogeneous arrangement, thanks to the special compacting process they have been subjected to.

The peculiarity of the material discloses in the patent consist of:
■ The particular yarns disposition which assure a controlled and homogeneous arrangement.
■ When the synthetic or cotton yarns release the compacted yarns they maintain a controlled and homogeneous arrangement filling the whole available cavity.

The described material may simply be winded up around the exhaust pipe, because during the first silencer's use, the synthetic yarns burns, so that the fiber glass increases its volume, filling the whole available cavity.

This product may be supplied precutted and/or preformed so that it can be quickly applied by unskilled personnel.

The homogenized yarns that have increased their volume, arranged inside the silencer, assure a great thermal and acoustic efficiency, together with a sure and even insulating action.

The material may be hybridized with other materials in order to satisfy the specific requirements of the purchaser.

The material may be combined with needled felt of low, medium and high density, so that it can be successfully used at various temperature up to 1200° C.

The above mentioned hybridization gives the possibility to commercialize a product adaptable to the purchasers' requirement.

The product density may be changed according to the specification.

In any case, formal and structural modification of the proposed solution may be made under the same inventive step as it is defined in the appended claims.

## Claims

1. Soundproofing and lagging material having two orthogonally overlapping fiber yarn wefts (1, 2), which are overlapped by two further fiber yarn layers with "V" arrangements, wherein the layers so overlapped are compacted and held together by sewing with synthetic or natural fiber, which, at a certain temperature, is able to release the compacted yarns which increase their volume.

2. The material according to claim 1, **characterized in that** said overlapped and compacted yarns are sewed parallel to the first fiber yarn weft (1).

3. The material according to claim 1 or 2, **characterized in that** said fiber yarn is a glass fiber yarn.

4. The material according to claim 1 or 2, **characterized in that** said fiber yarn is an aramid fiber yarn.

5. The material according to claim 1 or 2, **characterized in that** said fiber yarn is a synthetic fiber yarn.

6. The material according to claim 1 or 2, **characterized in that** said fiber yarn is a steel fiber yarn.

7. The material according to claim 1 or 2, **characterized in that** said fiber yarn is an inconel fiber yarn.

8. The material according to one of the preceding claims, said material being hybridized with other materials, in particular with needled felt of low, medium and high density.

## Patentansprüche

1. Schallschutz- und Isoliermaterial mit zwei senkrecht überlappenden Fasergarnschüssen (1, 2), die mit zwei weiteren Fasergarnschichten mit "V"-Anordnungen überdeckt sind, wobei die so überdeckten Schichten verdichtet sind und durch Vernähen mit synthetischer oder natürlicher Faser zusammengehalten werden, welche bei einer bestimmten Temperatur die verdichteten Garne freigeben kann, die ihr Volumen vergrößern.

2. Material nach Anspruch 1, **dadurch gekennzeichnet, dass** die überdeckten und verdichteten Garne parallel zu dem ersten Fasergarnschuss (1) vernäht sind.

3. Material nach Anspruch 1 oder 2, **dadurch gekennzeichnet, dass** das Fasergarn ein Glasfasergarn ist.

4. Material nach Anspruch 1 oder 2, **dadurch gekennzeichnet, dass** das Fasergarn ein Aramidfasergarn ist.

5. Material nach Anspruch 1 oder 2, **dadurch gekennzeichnet, dass** das Fasergarn ein synthetisches Fasergarn ist.

6. Material nach Anspruch 1 oder 2, **dadurch gekennzeichnet, dass** das Fasergarn ein Stahlfasergarn ist.

7. Material nach Anspruch 1 oder 2, **dadurch gekennzeichnet, dass** das Fasergarn ein Inconel-Fasergarn ist.

8. Material nach einem der vorhergehenden Ansprüche, wobei das Material mit anderen Materialien vermischt ist, insbesondere mit Nadelfilz mit geringer, mittlerer und hoher Dichte.

## Revendications

1. Matériau d'insonorisation et d'isolation thermique ayant deux trames de fils de fibre (1, 2) superposées orthogonalement, sur lesquelles sont superposées deux autres couches de fils de fibre disposées en « V », dans lequel les couches superposées de la sorte sont compactées et maintenues ensemble par couture avec une fibre naturelle ou synthétique, qui, à une certaine température, peut libérer les fils compactés pour augmenter leur volume.

2. Matériau selon la revendication 1, **caractérisé en ce que** lesdits fils compactés et superposés sont cousus parallèles à la première trame de fils de fibre (1).

3. Matériau selon la revendication 1 ou 2, **caractérisé en ce que** ledit fil de fibre est un fil de fibre de verre.

4. Matériau selon la revendication 1 ou 2, **caractérisé en ce que** ledit fil de fibre est un fil de fibre aramide.

5. Matériau selon la revendication 1 ou 2, **caractérisé en ce que** ledit fil de fibre est un fil de fibre synthétique.

6. Matériau selon la revendication 1 ou 2, **caractérisé en ce que** ledit fil de fibre est un fil de fibre d'acier.

7. Matériau selon la revendication 1 ou 2, **caractérisé en ce que** ledit fil de fibre est un fil de fibre Inconel.

8. Matériau selon l'une des revendications précédentes, ledit matériau étant hybridé avec d'autres matériaux, en particulier avec du feutre aiguilleté de faible, moyenne et forte densité.
